# EUROPEAN PATENT SPECIFICATION

(11) **EP 0 755 801 B1**
(45) Date of publication and mention of the grant of the patent: **18.08.1999**
(21) Application number: 96420218.8
(22) Date of filing: 28.06.1996
(51) Int. Cl.: B41M 5/24

(54) **Stabilizers for cyan dyes in dye - ablative element**
Stabilisatoren für Cyanfarbstoffe in Laserablationsaufzeichnungselement
Stabilisateurs pour colorants cyanes utilisés pour un élément d'enregistrement par ablation à laser

(30) Priority: 26.07.1995 US 1519; 21.03.1996 US 620055
(43) Date of publication of application: 29.01.1997
(73) Proprietor: EASTMAN KODAK COMPANY, Rochester, New York 14650-2201 (US)
(72) Inventor: Tutt, Lee William, c/o Eastman Kodak Co., Rochester, New York 14650-2201 (US); Chapman, Derek David, c/o Eastman Kodak Co., Rochester, New York 14650-2201 (US)
(74) Representative: Fevrier, Murielle Françoise E.

(56) References cited:
- EP-A- 0 636 493
- US-A- 5 219 823
- US-A- 5 399 459
- US-A- 5 429 909

## Description

This invention relates to the use of certain stabilizers for cyan dyes in a single-sheet laser dye-ablative recording element. In particular, this invention relates to laser dye ablation to generate optical masks and monochrome transparencies used in the fields of graphic arts and medical imaging.

In recent years, thermal transfer systems have been developed to obtain prints from pictures which have been generated electronically from a color video camera. According to one way of obtaining such prints, an electronic picture is first subjected to color separation by color filters. The respective color-separated images are then converted into electrical signals. These signals are then operated on to produce cyan, magenta and yellow electrical signals. These signals are then transmitted to a thermal printer. To obtain the print, a cyan, magenta or yellow dye-donor element is placed face-to-face with a dye-receiving element. The two are then inserted between a thermal printing head and a platen roller. A line-type thermal printing head is used to apply heat from the back of the dye-donor sheet. The thermal printing head has many heating elements and is heated up sequentially in response to the cyan, magenta or yellow signal. The process is then repeated for the other two colors. A color hard copy is thus obtained which corresponds to the original picture viewed on a screen. Further details of this process and an apparatus for carrying it out are contained in U.S. Patent 4,621,271.

Another way to thermally obtain a print using the electronic signals described above is to use a laser instead of a thermal printing head. In such a system, the donor sheet includes a material which strongly absorbs at the wavelength of the laser. When the donor is irradiated, this absorbing material converts light energy to thermal energy and transfers the heat to the dye in the immediate vicinity, thereby heating the dye to its vaporization temperature for transfer to the receiver. The absorbing material may be present in a layer beneath the dye and/or it may be admixed with the dye. The laser beam is modulated by electronic signals which are representative of the shape and color of the original image, so that each dye is heated to cause volatilization only in those areas in which its presence is required on the receiver to reconstruct the color of the original object. Further details of this process are found in GB 2,083,726A.

In one ablative mode of imaging by the action of a laser beam, an element with a dye layer composition comprising an image dye, an infrared-absorbing material, and a binder coated onto a substrate is imaged from the dye side. The energy provided by the laser drives off at least the image dye at the spot where the laser beam impinges upon the element. In ablative imaging, the laser radiation causes rapid local changes in the imaging layer thereby causing the material to be ejected from the layer. This is distinguishable from other material transfer techniques in that some sort of chemical change (e.g., bond-breaking), rather than a completely physical change (e.g., melting, evaporation or sublimation), causes an almost complete transfer of the image dye rather than a partial transfer. Usefulness of such an ablative element is largely determined by the efficiency at which the imaging dye can be removed on laser exposure. The transmission Dmin value is a quantitative measure of dye clean-out: the lower its value at the recording spot, the more complete is the attained dye removal.

Laser dye ablation is useful for the making of masks for the graphic arts industry, printing plates, printed circuit boards, and for generating medical imaging monochrome transparency images. These masks are used to mask light to another material or, in the case of medical images, to mask light to the eye, and are thus subjected to prolonged exposure to light. Photostability of the dyes is therefore a primary concern.

Cyan dyes have a tendency to fade within a relatively short period of time even on modest exposure to light from a "light table", i.e., a table having fluorescent bulbs to illuminate a film through a translucent plastic. Films subjected to light from a light table for a period of one week display definite visual dye fade and a hue shift toward yellow. Since yellow is a color which provides only low visual contrast, alignment of the film then becomes more difficult.

U.S. Patent 5,219,823 relates to a dye-donor element for laser-induced thermal dye transfer comprising a dye layer containing a cyanine infrared absorbing material and a nitrosonaphthol ferrous complex. However, there is no disclosure in this patent that the nitrosonaphthol ferrous complexes will specifically stabilize cyan image dyes or that such materials can be used in a laser dye-ablative process instead of a laser dye transfer process.

It is an object of this invention to provide a laser dye-ablative process which employs a stabilizer for cyan image dyes. It is another object of this invention to provide a stabilizer for cyan image dyes which is used in a dye-ablative recording element which does not contain a separate infrared-absorbing material.

These and other objects are achieved in accordance with this invention which relates to a process of forming a single color, ablation image comprising imagewise-exposing by means of a laser, in the absence of a separate receiving element, a dye-ablative recording element comprising a support having thereon a dye layer comprising a cyan image dye dispersed in a polymeric binder, the dye layer having a nitrosophenol or nitrosonaphthol ferrous complex associated therewith, optionally the dye layer also having an infrared-absorbing material associated therewith to absorb at a given wavelength of the laser used to expose the element, the cyan image dye not having substantial absorption at the wavelength of the laser used to expose the element, the laser exposure taking place through the dye side of said element, thereby imagewise-heating the dye layer and causing it to ablate, and removing the ablated material to obtain an image in said ablative recording element.

Another embodiment of the invention relates to a dye-ablative recording element comprising a support having thereon a dye layer comprising a cyan image dye dispersed in a polymeric binder, the element not containing a separate infrared-absorbing material, the dye layer having a nitrosophenol or nitrosonaphthol ferrous complex associated therewith.

In the present invention, the nitrosophenol or nitrosonaphthol ferrous complex which is added to a dye ablation film element results in increased fade resistance to light exposure while maintaining a reasonable dye removal rate (speed) and stain elimination (low Dmin level). The complex added may be in the form of a free salt or in the form of the counterion to an infrared-absorbing dye which may be present in the element. The latter form has the advantage that less material must be removed to reach Dmin, since the mass of the counterion is reduced which has to be ablated by elimination of inactive counterions for both stabilizer and IR-absorbing dye.

Any nitrosophenol or nitrosonaphthol ferrous complex may be employed in the invention. In a preferred embodiment, the nitrosophenol or nitrosonaphthol ferrous complex has the following formula: wherein:
X and Y each independently represents hydrogen, acetamido, alkyl or alkoxy of 1-4 carbon atoms, nitro, halogen or the atoms necessary to complete a fused, substituted or unsubstituted aromatic ring, with the proviso that when Y is an aromatic ring, then X can be hydrogen, acetamido, alkyl or alkoxy of 1-4 carbon atoms, nitro, or halogen; and
A represents a cation, such as ammonium, tetraalkyl ammonium, an alkali metal, 1-alkyl pyridinium, etc.

In another preferred embodiment of the invention, A represents tetraalkyl ammonium, Y is hydrogen and X represents methoxy. In another preferred embodiment, A represents tetraalkyl ammonium and either X or Y represents the atoms necessary to provide a fused naphthol ring.

Following are examples of the stabilizer complexes which may be employed in the invention:

In a preferred embodiment of the process of the invention, the infrared absorbing material is an infrared-absorbing dye and it and the nitrosophenol or nitrosonaphthol ferrous complex are in the dye layer.

The dye layer of the dye ablation element of the invention may also contain an ultraviolet-absorbing dye, such as a benzotriazole, a substituted dicyanobutadiene, an aminodicyanobutadiene, or any of those materials disclosed in Patent Publications JP 58/62651; JP 57/38896; JP 57/132154; JP 61/109049; JP 58/17450; or DE 3,139,156. They may be used in an amount of from about 0.05 to about 1.0 g/m².

The dye ablation elements of this invention can be used to obtain medical images, reprographic masks, printing masks, etc. The image obtained can be a positive or a negative image. The dye ablation or removal process can generate either continuous (photographic-like) or halftone images.

The invention is especially useful in making reprographic masks which are used in publishing and in the generation of printed circuit boards. The masks are placed over a photosensitive material, such as a printing plate, and exposed to a light source. The photosensitive material usually is activated only by certain wavelengths. For example, the photosensitive material can be a polymer which is crosslinked or hardened upon exposure to ultraviolet or blue light but is not affected by red or green light. For these photosensitive materials, the mask, which is used to block light during exposure, must absorb all wavelengths which activate the photosensitive material in the Dmax regions and absorb little in the Dmin regions. For printing plates, it is therefore important that the mask have high blue and UV Dmax. If it does not do this, the printing plate would not be developable to give regions which take up ink and regions which do not.

By use of this invention, a mask can be obtained which has enhanced stability to light for making multiple printing plates or circuit boards without mask degradation.

Any polymeric material may be used as the binder in the recording element employed in the invention. For example, there may be used cellulosic derivatives, e.g., cellulose nitrate, cellulose acetate hydrogen phthalate, cellulose acetate, cellulose acetate propionate, cellulose acetate butyrate, cellulose triacetate, a hydroxypropyl cellulose ether, an ethyl cellulose ether, etc., polycarbonates; polyurethanes; polyesters; poly(vinyl acetate); polystyrene; poly(styrene-co-acrylonitrile); a polysulfone; a poly(phenylene oxide); a poly(ethylene oxide); a poly(vinyl alcohol-co-acetal) such as poly(vinyl acetal), poly(vinyl alcohol-co-butyral) or poly(vinyl benzal); or mixtures or copolymers thereof. The binder may be used at a coverage of from about 0.1 to about 5 g/m².

In a preferred embodiment, the polymeric binder used in the recording element employed in the process of the invention has a polystyrene equivalent molecular weight of at least 100,000 as measured by size exclusion chromatography, as described in U.S. Patent 5,330,876.

A barrier layer may be employed in the laser ablative recording element of the invention if desired, as described in U.S. Patent 5,459,017.

To obtain a laser-induced, dye ablative image according to the invention, an infrared diode laser is preferably employed since it offers substantial advantages in terms of its small size, low cost, stability, reliability, ruggedness, and ease of modulation. In practice, before any laser can be used to heat a dye-ablative recording element, the element usually contains an infrared-absorbing material (unless the image dye absorbs at the wavelength of the laser), such as cyanine infrared-absorbing dyes as described in U.S. Patent 4,973,572, separate metal layers as described in U.S. Patent 5,256,506, or other materials as described in the following U.S. Patent Numbers: 4,948,777, 4,950,640, 4,950,639, 4,948,776, 4,948,778, 4,942,141, 4,952,552, 5,036,040, and 4,912,083. The laser radiation is then absorbed into the dye layer and converted to heat by a molecular process known as internal conversion. Thus, the construction of a useful dye layer will depend not only on the hue, transferability and intensity of the image dyes, but also on the ability of the dye layer to absorb the radiation and convert it to heat. The infrared-absorbing dye may be contained in the dye layer itself or in a separate layer associated therewith, i.e., above or below the dye layer. Preferably, the laser exposure in the process of the invention takes place through the dye side of the dye ablative recording element, which enables this process to be a single-sheet process, i.e., a separate receiving element is not required.

The dye layer of the dye-ablative recording element of the invention may be coated on the support or printed thereon by a printing technique such as a gravure process.

Any material can be used as the support for the dye-ablative recording element of the invention provided it is dimensionally stable and can withstand the heat of the laser. Such materials include polyesters such as poly(ethylene naphthalate); polysulfones; poly(ethylene terephthalate); polyamides; polycarbonates; cellulose esters; fluorine polymers; polyethers; polyacetals; polyclefins; and polyimides. The support generally has a thickness of from about 5 to about 200 µm. In a preferred embodiment, the support is transparent.

A thermal printer which uses a laser as described above to form an image on a thermal print medium is described and claimed in U.S. Patent 5,168,288.

Any cyan image dye can be used in the dye-ablative recording element employed in the invention provided it is **ablatable** by the action of the laser. Especially good results have been obtained with the following cyan dyes: or any of the cyan dyes disclosed in U.S. Patents 4,541,830, 4,698,651, 4,695,287, 4,701,439, 4,757,046, 4,743,582, 4,769,360, and 4,753,922. The above dyes may be employed singly or in combination with other dyes. The dyes may be used at a coverage of from about 0.05 to about 1 g/m² and are preferably hydrophobic.

The following examples are provided to illustrate the invention.

### Example 1

This example demonstrates that the nitrosophenol ferrous complex can be present in the form of a counterion for the infrared-absorbing dye.

Following are the structures of the various materials used in the examples:

Control elements were prepared by coating on a 100 µm poly(ethylene terephthalate) film an imaging layer of:

| | |
|---|---|
| nitrocellulose (1000-1500 sec.) | 0.604 g/m² |
| UV Dye | 0.172 g/m² |
| Yellow Dye | 0.284 g/m² |
| IF Dye-1 | 0.215 g/m² |
| Cyan Dyes 1-4 | amounts as shown in Table 1 |

The cyan dye level was varied to hold the nominal Status A red density to about 1.5 OD.

Elements according to the invention were prepared similar to the control elements except that they contained IF Dye-2 in the amount of 0.312 g/m². The infrared dye weight laydown was increased because of the counterion change to account for the increased molecular weight.

A sample of each film element was placed on a fluorescent light table for one week. The samples were positioned such that one half of each sample was protected from the light and the other half lay across the bulb region. The cyan dye fade was measured with an X-Rite Model 310 densitometer (X-Rite Corp., Grandville, MI) reading the Status A red absorbance.

The fade was expressed as the loss of red optical density as a percent change relative to the unexposed regions. A negative number implies a gain in optical absorption. The following results were obtained:

**TABLE 1**

| **ELEMENT CONTAINING: IR DYE/CYAN DYE (g/m**^{**2**}**)** | **LOSS OF RED OPTICAL DENSITY (%)** |
|---|---|
| IR Dye-1 (control)/Cyan Dye 1 (0.377 g/m²) | 25 |
| IR Dye-2/Cyan Dye 1 (0.377 g/m²) | 3 |
| IR Dye-1 (control)/Cyan Dye 2 (0.269 g/m²) | 22 |
| IR Dye-2/Cyan Dye 2 (0.269 g/m²) | -2 |
| IR Dye-1 (control)/Cyan Dye 3 (0.161 g/m²) | 89 |
| IR Dye-2/Cyan Dye 3 (0.161 g/m²) | 30 |
| IR Dye-1 (control)/Cyan Dye 4 (0.316 g/m²) | 60 |
| IR Dye-2/Cyan Dye 4 (0.316 g/m²) | 3 |

The above results show that significant improvements in minimizing loss of red optical density are obtained using various cyan dyes and an infrared-absorbing dye containing a nitrosophenol ferrous complex counterion in accordance with the invention.

### Example 2

This example illustrates the beneficial effects of the addition of a stabilizer to an element which does not contain any IR-absorbing dye which is employed in a dye-ablation process using a red laser.

A Control 2 element was prepared which is similar to the control element of Example 1 containing Cyan Dye 3, but without any IR Dye-1 present. Elements according to the invention were prepared similar to Control 2 except that they contained 0.097 g/m² of stabilizers S-1, S-2, S-3 and S-4. The light fade characteristics for 5 days on a light box were measured as in Example 1. The following results were obtained:

**TABLE 2**

| **ELEMENT CONTAINING STABILIZER** | **LOSS OF RED OPTICAL DENSITY (%)** |
|---|---|
| none (Control 2) | 88 |
| S1 | 36 |
| S2 | 42 |
| S3 | 20 |
| S4 | 50 |

The above results show that the addition of a stabilizer to an element without any IR-absorbing dye significantly improves the light fading characteristics.

### Example 3

This example illustrates the addition of a nitrosophenol ferrous complex to an ablation element which contains an IR-absorbing dye.

Control elements of Example 1 containing Cyan dyes 1 and 3 were prepared. Elements according to the invention were prepared similar to the control elements except that they contained stabilizer S-1 (0.097 g/m²). The light fade characteristics for one week on a light box were measured as in Example 1. The following results were obtained:

**TABLE 3**

| **ELEMENT CONTAINING:CYAN DYE/ STABILIZER** | **LOSS OF RED OPTICAL DENSITY (%)** |
|---|---|
| Cyan Dye 1/No stabilizer (control) | 22 |
| Cyan Dye 1/Stabilizer S-1 | 6 |
| Cyan Dye 3/No stabilizer (control) | 89 |
| Cyan Dye 3/Stabilizer S-1 | 33 |

The above results show that adding a stabilizer as a separate salt to the ablation element significantly improves the light fading characteristics.

### Example 4

The four elements of Example 3 were laser ablated to remove all dye where the laser irradiated, using nine 700 milliwatt lasers with an average power at the focal plane of 550 milliwatts. A 53 cm drum was rotated at 1040 rev/min to give an energy of 583 mJ/cm². This resulted in an image region that was essentially cleaned out down to the base and was only 0.02 above the lowest ultraviolet Dmin achieved at higher powers.

The optical density was measured in the ultraviolet because the films were more sensitive to cleanout at ultraviolet. The ultraviolet Dmin was measured on an X-Rite Model 361T densitometer. The Status A red Dmin values were all 0.05 and the UV Dmax values were all 2.77±0.11. The following results were obtained:

**TABLE 4**

| **ELEMENT CONTAINING: CYAN DYE/ STABILIZER** | **UV Dmin** |
|---|---|
| Cyan Dye 1/No stabilizer (control) | 0.12 |
| Cyan Dye 1/Stabilizer S-1 | 0.14 |
| Cyan Dye 3/No stabilizer (control) | 0.12 |
| Cyan Dye 3/Stabilizer S-1 | 0.15 |

The above results show a very minor change in the ultraviolet Dmin upon addition of the stabilizer. The impact on the speed (amount of light necessary to achieve Dmin) of ablation is therefore small. Thus, the addition of a stabilizer to the element does not have any appreciable adverse effects.

## Claims

1. A process of forming a single color, ablation image comprising imagewise-exposing, by means of a laser, in the absence of a separate receiving element, a dye-ablative recording element comprising a support having thereon a dye layer comprising a cyan image dye dispersed in a polymeric binder, said dye layer having a nitrosophenol or nitrosonaphthol ferrous complex associated therewith, optionally said dye layer also having a separate infrared-absorbing material associated therewith to absorb at a given wavelength of said laser used to expose said element, when said cyan image dye does not have substantial absorption at the wavelength of said laser used to expose said element, said laser exposure taking place through the dye side of said element, thereby imagewise-heating said dye layer and causing it to ablate, and removing the ablated material to obtain an image in said ablative recording element.

2. The process of Claim 1 wherein said infrared absorbing material and said nitrosophenol or nitrosonaphthol ferrous complex are in said dye layer.

3. The process of Claim 1 wherein said nitrosophenol or nitrosonaphthol ferrous complex has the following formula: wherein:
X and Y each independently represents hydrogen, acetamido, alkyl or alkoxy of 1-4 carbon atoms, nitro, halogen or the atoms necessary to complete a fused, substituted or unsubstituted aromatic ring, with the proviso that when Y is an aromatic ring, then X can be hydrogen, acetamido, alkyl or alkoxy of 1-4 carbon atoms, nitro, or halogen; and
A represents a cation.

4. The process of Claim 3 wherein A represents tetraalkyl ammonium, Y is hydrogen and X represents methoxy.

5. The process of Claim 3 wherein A represents tetraalkyl ammonium and either X or Y represents the atoms necessary to provide a fused naphthol ring.

6. The process of Claim 1 wherein said infrared-absorbing material is a dye having a counter ion.

7. The process of Claim 6 wherein said nitrosophenol or nitrosonaphthol ferrous complex is the counter ion for said infrared-absorbing dye.

8. The process of Claim 1 wherein said element does not contain a separate infrared-adsorbing material.

9. A dye-ablative recording element comprising a support having thereon a dye layer comprising a cyan image dye dispersed in a polymeric binder, said element not containing a separate infrared-absorbing material, said dye layer having a nitrosophenol or nitrosonaphthol ferrous complex associated therewith.

10. The element of Claim 9 wherein said nitrosophenol or nitrosonaphthol ferrous complex is in said dye layer.

11. The element of Claim 9 wherein said nitrosophenol or nitrosonaphthol ferrous complex has the following formula: wherein:
X and Y each independently represents hydrogen, acetamido, alkyl or alkoxy of 1-4 carbon atoms, nitro, halogen or the atoms necessary to complete a fused, substituted or unsubstituted aromatic ring, with the proviso that when Y is an aromatic ring, then X can be hydrogen, acetamido, alkyl or alkoxy of 1-4 carbon atoms, nitro, or halogen; and
A represents a cation.

## Patentansprüche

1. Verfahren zur Bildung eines einfarbigen Ablationsbildes, umfassend das bildweise Belichten mittels eines Lasers in Abwesenheit eines gesonderten Empfangselementes eines Farbstoff-ablativen Aufzeichnungselementes, welches einen Träger umfaßt, der darauf eine Farbstoffschicht aufweist, die einen Cyanbild-Farbstoff in einem polymeren Bindemittel dispergiert umfaßt, wobei der Farbstoffschicht ein Nitrosophenol- oder Nitrosonaphtholeisen(II)-Komplex zugeordnet ist, wobei der Farbstoffschicht gegebenenfalls auch ein gesondertes Infrarot-absorbierendes Material zugeordnet ist, um bei einer gegebenen Wellenlänge des Lasers, der zur Belichtung des Elements verwendet wird, zu absorbieren, wenn der Cyanbild-Farbstoff keine wesentliche Absorption bei der Wellenlänge des Lasers aufweist, der zur Belichtung des Elementes verwendet wird, wobei die Laserbelichtung durch die Farbstoffseite des Elements stattfindet, wodurch die Farbstoffschicht bildweise erwärmt wird und veranlaßt wird, eine Ablation einzugehen, und das Entfernen des eine Ablation eingegangenen Materials, um ein Bild in dem ablativen Aufzeichnungselement zu erhalten.

2. Verfahren nach Anspruch 1, in welchem das Infrarot-absorbierende Material und der Nitrosophenol- oder Nitrosonaphtholeisen(II)-Komplex in der Farbstoffschicht vorliegen.

3. Verfahren nach Anspruch 1, in welchem der Nitrosophenol- oder Nitrosonaphtholeisen(II)-Komplex die folgende Formel aufweist: in der:
X und Y jeweils unabhängig Wasserstoff, Acetamido, Alkyl oder Alkoxy mit 1 - 4 Kohlenstoffatomen, Nitro, Halogen oder die Atome darstellen, die notwendig sind, um einen kondensierten, substituierten oder unsubstituierten aromatischen Ring zu vervollständigen, mit der Maßgabe, daß dann, wenn Y ein aromatischer Ring ist, X Wasserstoff, Acetamido, Alkyl oder Alkoxy mit 1 - 4 Kohlenstoffatomen, Nitro oder Halogen sein kann; und
A ein Kation darstellt.

4. Verfahren nach Anspruch 3, in welchem A Tetraalkylammonium darstellt, Y Wasserstoff ist und X Methoxy darstellt.

5. Verfahren nach Anspruch 3, in welchem A Tetraalkylammonium darstellt und entweder X oder Y die Atome darstellt, die notwendig sind, um einen kondensierten Naphtholring zu liefern.

6. Verfahren nach Anspruch 1, in welchem das Infrarot-absorbierende Material ein Farbstoff mit einem Gegenion ist.

7. Verfahren nach Anspruch 6, in welchem der Nitrosophenol- oder Nitrosonaphtholeisen(II)-Komplex das Gegenion für den Infrarot-absorbierenden Farbstoff ist.

8. Verfahren nach Anspruch 1, in welchem das Element kein gesondertes Infrarot-absorbierendes Material enthält.

9. Farbstoff-ablatives Aufzeichnungselement, das einen Träger umfaßt, der darauf eine Farbstoffschicht aufweist, welche einen Cyanbild-Farbstoff in einem polymeren Bindemittel dispergiert umfaßt, wobei das Element kein gesondertes Infrarot-absorbierendes Material enthält, wobei der Farbstoffschicht ein Nitrosophenol- oder Nitrosonaphtholeisen(II)-Komplex zugeordnet ist.

10. Element nach Anspruch 9, in welchem der Nitrosophenol- oder Nitrosonaphtholeisen(II)-Komplex in der Farbstoffschicht vorliegt.

11. Element nach Anspruch 9, in welchem der Nitrosophenol- oder Nitrosonaphtholeisen(II)-Komplex die folgende Formel aufweist: in der:
X und Y jeweils unabhängig Wasserstoff, Acetamido, Alkyl oder Alkoxy mit 1 - 4 Kohlenstoffatomen, Nitro, Halogen oder die Atome darstellen, die notwendig sind, um einen kondensierten, substituierten oder unsubstituierten aromatischen Ring zu vervollständigen, mit der Maßgabe, daß dann, wenn Y ein aromatischer Ring ist, X Wasserstoff, Acetamido, Alkyl oder Alkoxy mit 1 - 4 Kohlenstoffatomen, Nitro oder Halogen sein kann; und
A ein Kation darstellt.

## Revendications

1. Procédé de formation d'une image monochrome par ablation comprenant l'exposition, en conformité avec l'image, au moyen d'un laser et en l'absence d'un élément récepteur distinct, d'un élément d'enregistrement fonctionnant par ablation du colorant, comprenant un support revêtu d'une couche de colorant comprenant un colorant d'image cyan dispersé dans un liant polymère, un complexe ferreux nitrosophénol ou nitrosonaphtol étant associé à ladite couche de colorant, une substance absorbant dans l'infrarouge distincte étant éventuellement associée à ladite couche de colorant, afin d'absorber à la longueur d'onde déterminée du laser utilisé pour exposer ledit élément, lorsque ledit colorant d'image cyan n'absorbe pratiquement pas à la longueur d'onde du laser utilisé pour exposer ledit élément, ladite exposition au laser étant faite du côté de l'élément portant le colorant, ce qui permet de chauffer ladite couche de colorant conformément à l'image et provoque son ablation, et permet également d'éliminer le matériau ayant subi l'ablation pour obtenir une image dans ledit élément d'enregistrement fonctionnant par ablation.

2. Procédé selon la revendication 1, dans lequel ladite substance absorbant dans l'infrarouge et ledit complexe ferreux nitrosophénol ou nitrosonaphtol sont incorporés dans ladite couche de colorant.

3. Procédé selon la revendication 1, dans lequel ledit complexe ferreux nitrosophénol ou nitrosonaphtol est représenté par la formule suivante : où :
X et Y représentent chacun indépendamment l'hydrogène, un groupe acétamido, alkyle ou alcoxy de 1 à 4 atomes de carbone, nitro, un halogène ou les atomes nécessaires pour compléter un cycle aromatique condensé substitué ou non, à la condition que lorsque Y est un cycle aromatique, X puisse être l'hydrogène, un groupe acétamido, alkyle ou alcoxy de 1 à 4 atomes de carbone, nitro ou un halogène ; et
A représente un cation.

4. Procédé selon la revendication 3, dans lequel A représente un groupe tétraalkyl ammonium, Y est l'hydrogène et X représente un groupe méthoxy.

5. Procédé selon la revendication 3, dans lequel A représente un groupe tétraalkyl ammonium et soit X soit Y représente les atomes nécessaires pour former un cycle naphtol condensé.

6. Procédé selon la revendication 1, dans lequel ladite substance absorbant dans l'infrarouge est un colorant comprenant un contre-ion.

7. Procédé selon la revendication 6, dans lequel ledit complexe ferreux nitrosophénol ou nitrosonaphtol est le contre-ion pour ledit colorant absorbant dans l'infrarouge.

8. Procédé selon la revendication 1, dans lequel ledit élément ne contient pas de substance absorbant dans l'infrarouge distincte.

9. Elément d'enregistrement par ablation de colorant comprenant un support revêtu d'une couche de colorant comprenant un colorant d'image cyan dispersé dans un liant polymère, ledit élément ne contenant pas de substance absorbant dans l'infrarouge distincte, un complexe ferreux nitrosophénol ou nitrosonaphtol étant associé à ladite couche de colorant.

10. produit selon la revendication 9, dans lequel ledit complexe ferreux nitrosophénol ou nitrosonaphtol se trouve dans ladite couche de colorant.

11. produit selon la revendication 9, dans lequel ledit complexe ferreux nitrosophénol ou nitrosonaphtol est représenté par la formule suivante : où :
X et Y représentent chacun indépendamment l'hydrogène, un groupe acétamido, alkyle ou alcoxy de 1 à 4 atomes de carbone, nitro, un halogène ou les atomes nécessaires pour compléter un cycle aromatique condensé substitué ou non, à la condition que lorsque Y est un cycle aromatique, X puisse être l'hydrogène, un groupe acétamido, alkyle ou alcoxy de 1 à 4 atomes de carbone, nitro ou un halogène ; et
A représente un cation.
